

## UNITED STATES PATENT OFFICE.

HARRY LE B. GRAY, OF ROCHESTER, NEW YORK, ASSIGNOR TO EASTMAN KODAK COMPANY, OF ROCHESTER, NEW YORK, A CORPORATION OF NEW YORK.

## METHOD OF INCREASING THE UNIFORMITY OF CELLULOSE ESTERS.

No Drawing.

Application filed August 25, 1927. Serial No. 215,519.

This invention relates to methods of increasing the uniformity of cellulose esters. One object of the invention is to provide a method which is relatively simple and inexpensive to carry out, and yet mixes the ingredients so thoroughly that esters of great uniformity, especially in their solubilities, are produced. Another object of the invention is to impregnate the cellulosic material or fibers, prior to esterification, very uniformly, even when the proportion of acylating liquid, relative to the cellulose, is small. Other objects will hereinafter appear.

It is highly desirable in the manufacture of cellulose esters of organic acids to obtain products which are of high uniformity in their solubility. This uniformity is greatly dependent upon the thoroughness with which the acylating liquid is mixed with the cellulosic fibers prior to esterification. For example, in making cellulose acetate, it is desirable to obtain uniform acetylation throughout all parts of the fibers, so that all of such parts will be soluble in chloroform, and ultimately in acetone. This avoids the presence of insoluble particles which cause a hazy appearance in solutions or films made from the esters.

One of the principal well known ways of mixing the cellulosic material and the reacting liquid is to immerse the cellulosic fibers in an excess of the liquid. Sometimes the excess of liquid is allowed to remain during the esterification reaction. At other times the excess of liquid is removed, say by pressure, and only a smaller proportion of the liquid stays behind in the fibers to effect the esterification. It has been found that there is a noticeable tendency for non-uniform mixing to occur under these conditions. Each fiber of the cellulosic material is not fully wetted with the organic esterifying liquid, and a non-uniform product results, from which hazy films are produced. The lack of uniformity may be partly due to air that is trapped along the fibers in the form of small bubbles, or to surface repellency of the fibers toward the esterifying liquid.

I have found that esters of high uniformity may be prepared and the effects of air bubbles and surface repellency may be successfully combatted by mixing the acylating liquid with a volatile, substantially non-re-

acting solvent vehicle, incorporating this mixture with the cellulosic fibers and then removing the vehicle by evaporation or distillation under a vacuum. In the preferred form of my invention the fibers are first placed under a vacuum, and then the mixture of acylating liquid and the liquid vehicle are run into the fibers while the vacuum is maintained. Then the vehicle is removed under vacuum, the vacuum is broken and esterification allowed to proceed under normal conditions at or above atmospheric pressure.

My invention is applicable in connection with any of the cellulosic fibers which are useful in making cellulose esters of organic acids. Since cellulose acetate is at present the most important of such esters, I shall describe, by way of illustration, the use of acetylating liquids in carrying out my process; but it will be understood that my invention is applicable to any similar organic acetylating liquids, such, for instance, as those described in the applications of Hans T. Clarke and Carl J. Malm, Serial Nos. 179,- 176 and 179,177 for "process of making organic esters of cellulose containing acyl groups having more than two carbon atoms", and "process of making cellulose esters of organic acids", both filed March 28th, 1927. Instances of such liquids include acetic anhydrid with any of lauric, myristic, palmitic or stearic acid; chloracetic anhydrid with stearic or formic acid.

For the liquid vehicle any of the relatively inexpensive volatile organic solvents, which do not substantially react with the other ingredients of the reaction mixture, may be employed. Chloroform or ether may be successfully used, for instance. The removal of the liquid vehicle from the mixture under a vacuum by evaporation is carried out at a temperature sufficiently low to hold back the esterification reaction during the removal of the vehicle.

My present invention is of especial usefulness in carrying out the process set forth in the prior application of myself and C. J. Staud, Serial No. 196,999, filed July 6th, 1927 for "process of making chloroform-soluble cellulose acetate." In that process the cellulosic material is mixed with a relatively small proportion of acylating liquid. It is particularly difficult to mix such a small proportion of such liquid with the fibers to

obtain the necessary uniformity. My present method enables even very small amounts of the esterifying liquid, such as acetic anhydrid, to be distributed with the 5 utmost uniformity throughout the cellulosic fibers.

For example 100 parts by weight of clean cotton fibers, say filter cotton, are placed under a vacuum of 14 to 40 millimeters of 10 mercury. There is then added to the fibers, while they are still under a vacuum, a mixture of 220 parts of acetic anhydrid (94% strength), 1800 parts of chloroform by weight, and .25 parts by weight of sulfuric 15 acid and .25 parts by weight of phosphoric acid. The liquid mixture, including the chloroform, is sufficient in quantity to thoroughly and uniformly wet every fiber. Then while the vacuum is kept up the 20 chloroform is allowed to evaporate, and its vapors are recovered by condensation or absorption. In place of the chloroform, 850 parts by weight of ethyl ether can be employed, but the chloroform is more readily 25 removed, particularly at or about room temperature. After the chloroform is removed, the vacuum is broken, and the acetylation conducted as described in said application, Serial No. 196,999. The fibers, uniformly 30 moist with the acetic anhydrid and catalyst, are allowed to stand in a closed vessel at room temperature until the reaction is finished. This is indicated when test samples from the reaction mixture fully dissolve in 35 pure chloroform. The end of the reaction may likewise be found by examining test specimens by polarized light, using a microscope arranged with crossed Nicol's prisms and a selenite plate so located as to give the 40 most brilliant red field. During the acetylation, the fibers change from brilliant yellow to a deep red or blue, depending upon the position of the fibers relative to the plane of polarization of the light. The fully acetylated 45 fibers, under these conditions, retain their fibrous appearance without dissolving, or coming together so as to be difficultly manipulatable in the subsequent stages of treatment.

50 Having thus described my invention, what I claim as new and desire to secure by Letters Patent is:

1. The method of making cellulose esters

of organic acids which comprises the steps 55 of thoroughly mixing the cellulosic material to be esterified with an inert volatile organic liquid vehicle having dissolved therein the amount of acylating agent for the reaction and also carrying a catalyst, evaporating said vehicle under a vacuum 60 from the mixture, thereby leaving said acylating agent and catalyst uniformly distributed throughout said fibers, breaking the vacuum and conducting the esterification reaction. 65

2. The method of making cellulose esters of organic acids which comprises the steps of placing the cellulosic fibers to be esterified under a vacuum, thoroughly mixing said fibers while maintaining a vacuum, with 70 an inert volatile organic liquid vehicle having dissolved therein the amount of acylating agent for the reaction and also carrying a catalyst, evaporating said vehicle under vacuum from the mixture, thereby leaving 75 said agent and catalyst uniformly distributed throughout said fibers, breaking the vacuum and conducting the esterification reaction.

3. The method of making cellulose acetate 80 which comprises the steps of thoroughly impregnating cellulosic fibers with an inert volatile organic liquid vehicle having dissolved therein the amount of acetic anhydrid for the reaction and a catalyst, evaporating said vehicle under vacuum from the mixture, thereby leaving said anhydrid and catalyst uniformly distributed throughout 85 said fibers, breaking the vacuum and conducting the acetylation. 90

4. The method of making cellulose acetate which comprises the steps of placing the cellulosic fibers to be esterified under a vacuum, mixing said fibers while maintaining a vacuum, with an inert volatile organic liquid vehicle having dissolved therein the amount of acetic anhydrid for the reaction and also carrying a catalyst, evaporating said vehicle under vacuum from the mixture, thereby leaving said anhydrid and catalyst uniformly distributed throughout 95 said fibers, breaking the vacuum and conducting the acetylation. 100

Signed at Rochester, New York, this 19th day of Aug., 1927.

HARRY LE B. GRAY.